

1

3,290,234

## ELECTRODEPOSITION OF PALLADIUM

Edward A. Parker, Cranston, R.I., and Alfred M. Weisberg, Chicago, Ill., assignors to Technic, Inc., Cranston, R.I., a corporation of Rhode Island  
No Drawing. Filed Oct. 29, 1963, Ser. No. 319,661  
4 Claims. (Cl. 204—47)

The present invention relates to the electrodeposition of palladium and, more particularly, to the preparation of palladium electroplates possessing bright, smooth, and lustrous surfaces even at heavy thicknesses.

The known methods of depositing palladium from baths used in the prior art suffer various difficulties. Among these may be mentioned instability of the bath, buildup of deleterious side-products, hazy deposits in all but thin coatings, and low deposition rates.

It is therefore a primary object of the present invention to provide a solution from which palladium may be electrically deposited in a convenient manner whereby a plate is produced which is bright, smooth, and lustrous.

It is a further object of the present invention to provide a solution from which palladium may be electrically deposited at room temperature.

It is another object of the present invention to provide a solution from which palladium may be electrically deposited in thick smooth plates at relatively rapid rates.

It is still another object of this invention to provide a process for the aqueous electrodeposition of palladium from a neutral solution.

Other objects, advantages, and results of the present invention will be apparent to anyone skilled in the knowledge of this art.

We have discovered that these several advantages can be secured by electroplating from a bath containing palladium in the form of a complex in solution in the concentration in the range of 2-10 grams of metal per liter of solution in the form of a complex of a cyclic-alkylene-moiety diamine tetraacetic acid, for example, selected from the group consisting of cyclopropylene, cyclobutene, cyclopentene and cyclohexane, N,N<sup>1</sup>-tetraacetic acid. Also, it should be understood that the acetic acid moiety can be replaced by propionic acid moiety. More generally stated, the chelate complex may be defined as follows:



wherein the X is a cyclic aliphatic moiety having N's on adjacent carbon atoms as the diamine wherein acetic acid moieties replace hydrogens to form the amino acid chelating compound.

The advantage of these cyclic moieties is that the chelate formed with palladium is strong enough to hold the palladium in solution. In other forms of chelate it is not stable and is reduced to the elemental state.

It is known that palladium forms very strong chelates with aminopolycarboxylic acids. With common ligands of this type, such as ethylenediamine tetraacetic acid, the reducing power of the amino acid moiety is sufficient to reduce aqueous solutions of the palladium chelate to the elemental state. It has been found that this reduction reaction is accelerated by a low pH.

We have discovered, however, that the aqueous solution of a palladium N,N<sup>1</sup> cyclohexanediamine tetraacetic acid chelate is stable over the pH range of 4 to 12. Below pH 4 the limited solubility of the chelate

2

practically precludes its use as an effective electroplating solution.

Similarly, other diamines having a cyclic moiety between the nitrogens are stable in the broad pH range and are responsive to electric currents so that our fundamental conditions are preserved, namely, the palladium is kept in solution and is electro-deposited, and contaminating metal ions are precipitated.

The palladium metal concentration in this bath may be varied over wide limits, but a practical range for clean, mirror bright plates is 2 to 10 grams of metal per liter.

The temperature of this novel bath may be varied from 20° to 65° C. It has been found, however, that room temperature operation is a facile manner to obtain bright, stress-free deposits.

The pH of this bath is not critical between the limits of 4.0 and 12.0. A neutral bath with a pH range of 6 to 8 has been found to be very useful. The use of buffer materials, such as mono-potassium phosphate, not only serve to control the pH but also act as effective conductivity salts.

The buffer materials are useful not only for pH control but also as precipitants of contaminating metal ions. Generally, since plating is done on a base metal, it is a quite common experience to have traces of nickel, copper, iron and the like appear in the bath as a result of drag-in, etc. Too much contamination by such metal ions in solution will ruin the usefulness of the bath because the contaminating metal will plate out. Under the conditions we maintain, particularly, the strong complex of palladium, acid pH, and soluble phosphate in solution, without other acids having good complexing properties, contaminating metals are precipitated as they reach the plating bath.

Cathode current efficiencies are quite high which tends to eliminate any stress due to hydrogen embrittlement. A current efficiency approaching 100% may be obtained at a current density of 10 amperes per square foot. Higher metal concentrations permit the use of higher current densities. A similar result may also be obtained with the aid of agitation.

Insoluble anodes of stainless steel, platinum, or carbon may be used. It is important to avoid anodes of any kind which, because of the chemistry of the solution, are likely to contribute undesirable ions in the plating bath. The palladium metal concentration may be maintained on the basis of ampere hours of use of the bath and by the addition of palladium as oxide or cyclohexene diamine tetraacetic acid salt to replace losses. With the removal of substantial amounts of palladium from the bath, it is possible to avoid accumulation of excess free chelating agent in the bath by the addition of palladium oxide to be dissolved and to form the chelate.

The following examples illustrate the application of these principles to the bath composition and operation, and the exemplification which follows should not be construed as limiting the invention but merely illustrates its spirit and scope.

## Example I

60 5 grams of palladium as the palladium chelate of N,N<sup>1</sup> cyclohexane-diamine tetra-acetic acid  
60 grams of mono-potassium phosphate.

Water to one liter.

This bath when used at 50° C. and a current density of 5 ASF will produce a brilliant palladium electrodeposit.

## Example II

70 10 grams of palladium as the palladium chelate of N,N<sup>1</sup> cyclohexane-diamine tetra-acetic acid  
40 grams of mono-potassium phosphate  
30 grams of citric acid

Water to one liter.

When this solution is adjusted to pH 5.0, pure, mirror bright palladium electrodeposits may be obtained at room temperature with a current density of 5 ASF.

*Example III*

Using the formulae of Examples I and II, the chelate of cyclopropylene diamine tetra-acetic acid is useful.

*Example IV*

Using the formulae of Examples I and II, the palladium chelate of cyclobutene N-N' diamine tetra-acetic acid is useful.

Generally, a palladium concentration in the range of about 2 grams to about 10 grams of the palladium metal per liter of solution is most useful.

In carrying out plating operations using these baths, it is to be noted that good plating technique is to be followed. That is, ampere hours of use of the bath are measured, the temperature of the bath is controlled reasonably closely to the recommended levels, it is agitated, pH of the bath is followed and adjustment within reasonable tolerance of recommended levels is made and, generally, clean plating techniques are followed. Regardless of the care with which plating operations are carried on in a working installation, it may be noted that when a base metal such as iron has been plated with copper and nickel, whether the article be costume jewelry or a piece of scientific apparatus, the best techniques will still produce situations in which the plating baths become contaminated with iron, copper, nickel, etc. Since it is not the desire of the operator to plate palladium alloys, this bath automatically corrects such contamination conditions, because by maintaining the palladium in platable condition in the form of the highly selective chelates described and maintaining acid conditions in the bath at a level such that the phosphates of iron, copper, nickel and the like are directly precipitated as such, the contaminants are automatically precipitated. Hence, the bath, for all practical purposes, is a bath of pure palladium chelate. For good operating technique, it is desirable occasionally to filter the bath.

The foregoing examples illustrating working formulas for the deposition of bright palladium coatings specifically indicate an operating pH of 5. It is to be understood that operable pH within the range of 4-12 can be used with the palladium chelate solutions identified but the preferred range is slightly on the acid side, 5-6-7.

One of the reasons for the acid pH operation is to maintain conditions in the bath such that contaminating metal ions will be precipitated as their phosphates. Accordingly, all of the examples may be actually read as pH operation 4-12, preferred being 5-6-7. Similarly, where the specific examples show the cyclohexene diamine acetic acid compound as the chelating agent, it should be understood that substantially the same results are obtained when the cyclopropene, cyclobutene, cyclopentene are used, because the stability of these compounds is of the same order of magnitude as the cyclohexene.

What is claimed is:

1. A bath for electro-plating palladium consisting essentially of the palladium chelate of an N,N<sup>1</sup>-cyclic alkylene diamine tetraacetic acid dissolved in water with a phosphate conductor, and a buffer to hold pH at a given level in the range about 4-12.
2. A bath in accordance with claim 1 in which the palladium compound is the palladium chelate of cyclo hexane diamine tetraacetic acid and the bath is buffered to a pH in the range from about 4 to about 12.
3. A bath in accordance with claim 2 in which the concentration of palladium compound maintained in the solution is in the range from about 2 grams to about 10 grams of metal per liter.
4. A method of electro-plating palladium to form heavy, clean, stress-free, bright plates which comprises providing an aqueous solution of palladium in the form of a chelate stable under plating conditions, the said chelate consisting essentially of palladium chelates of cyclic aliphatic N,N<sup>1</sup>-diamine tetraacetic compounds in the presence of anions in said solution suitable for precipitating contaminating metals but insufficient to precipitate the palladium, said solution being maintained at a pH in the range from 4-12, and passing an electric current through said solution from an anode to a cathode to be coated.

References Cited by the Examiner

UNITED STATES PATENTS

- |           |         |                  |       |        |
|-----------|---------|------------------|-------|--------|
| 2,335,821 | 11/1943 | Wise et al.      | ----- | 204-47 |
| 2,452,308 | 10/1948 | Lambros          | ----- | 204-47 |
| 2,984,595 | 5/1961  | Schumpelt et al. | ----- | 204-47 |

JOHN H. MACK, Primary Examiner.

G. KAPLAN, Assistant Examiner.